

## UNITED STATES PATENT OFFICE.

JOSEPH H. WALLACE, OF STAMFORD, CONNECTICUT, ASSIGNOR TO PINE WASTE PRODUCTS, INC., OF NEW YORK, N. Y., A CORPORATION OF DELAWARE.

## WOOD-PULP MATERIAL.

As Drawing.

Application filed August 25, 1920. Serial No. 403,985.

To all whom it may concern:

Be it known that I, JOSEPH H. WALLACE, a citizen of the United States, and a resident of Stamford, county of Fairfield, and State 5 of Connecticut, have invented certain new and useful Improvements in Wood-Pulp Material, of which the following is a specification.

This invention relates to the materials 10 used for the manufacture of paper pulp, and has for its object to provide an efficient and at the same time a relatively cheap material for paper pulp which can be produced by inexpensive methods and in 15 practically unlimited quantities.

The manufacture of paper pulp from wood by chemical processes involves what may be called a fractional or selective attack upon the wood components; the object 20 being to produce a disintegration or solution of certain relatively less resistant components while leaving unattacked or unacted on certain relatively resistant components or "cellulose." The yield and 25 quality of product depend largely upon the care with which the operation is performed; upon the observance of conditions which have been empirically established by long 30 practice. The greater the exactitude with which these conditions can be observed, the better the results; but, for various reasons, the ordinary practice is not standardized to the degree which is desirable. It is an object of the present invention to promote 35 accuracy and uniformity of operation by the provision of a standardized raw material; thereby facilitating standardization of the whole operation. With a standardized raw material there is no difficulty in using 40 solutions of exact and standard composition; or of employing exact temperatures and an exact time of digestion.

Wood is a variable material; and particularly as regards moisture content and the 45 content and character of "extractives"—non-fibrous components. These variables much influence the operation in pulp making; it being, for example, necessary to correct the strength of the solutions used for 50 the greater or less amount of water brought in by the wood. Again, in the alkaline processes, with the production of raw materials for which the present invention is 55 chiefly, though not exclusively, concerned, variations in the amount and character of

the acid resins of the wood make much difference in the activity of an alkali solution of given strength.

In the soda and sulfate processes, chipped wood in fragments long enough to give the 60 desired length of fiber, is heated in a digester under pressure with an alkaline liquid to give a disintegration and solution of the non-cellulose portion of the woody fiber, or "lignin", and a removal of the 65 various extractives, including resins. Naturally, the less acid material in the chips, the more of the alkali is available for resolution of lignin, and vice versa. With some woods, otherwise well adapted for pulp 70 making, as with southern pine, the amount of acid resins present is so great as to render treatment of such wood by the ordinary alkaline processes very difficult. With any resinous wood, however, the 75 amount of resin varies from log to log; and in the same log, or chip, from point to point. Variations in moisture content accompany variations in resin content. Resinous woods, and resinous parts of wood, absorb less moisture than non-resinous or less resinous woods or parts thereof.

In all alkaline processes, after the completion of the digestion, or the pulp making 80 operation proper, the black liquor is withdrawn, evaporated, charred and burnt in order to recover the alkali for reuse; and much of the economy of operation depends upon the efficiency of the alkali-recovery. The process is, therefore, an integral one; 85 conditions affecting alkali recovery must be considered as well as, and in connection with, conditions affecting the digestion only. In the digestion some resin is desirable as 90 its presence facilitates the action; and in the black liquor it is still more desirable as adding fuel value to the residues, thereby aiding materially in the final combustion prior to recovering alkali. It is not however in either case necessary or desirable 95 that it be an acid resin.

The extractives which may be recovered from coniferous wood with the aid of volatile solvents, such as alcohol, gasoline, benzol, the natural distillate known as "solvent", spirits of turpentine, etc., are many and of varied nature; but in a general way it may be said that they consist of acid, more or less crystalline resins of the nature of ordinary colophony or rosin, and neutral 110

resins, some more or less crystalline and hard and some amorphous and soft, and of various terpenes, some volatile and some not. On extracting such a wood with a solvent, the extraction process will be found to take place in two phases; an initial extraction taking place quite readily and giving solutions containing large amounts of dissolved matter and a secondary extraction which is slow and gives solutions much less charged with solutes. With southern pine, in the first stage the resins extracted are largely of a hard nature and have a high acid value, while in the second stage, the matter removed is more of a neutral, soft and amorphous nature. Similarly, the first stage removes most of the turpentine, pine oil and intermediate liquid products while the terpenes removed in the second stage are largely amorphous, gummy materials.

In the present invention, advantage is taken of the stated facts. Coniferous wood of any kind is chipped into pieces of the size of those wanted for paper pulp mill work, say from  $\frac{5}{8}$  to  $\frac{7}{8}$  inch in length, by  $\frac{1}{2}$  to  $\frac{1}{4}$  inches in width and  $\frac{1}{8}$  to  $\frac{3}{16}$  inch in thickness and these are submitted to a brief extraction with a suitable solvent; the extraction being merely long enough to bring the residual resin to a standard amount. Pine poor in resin needs but little extraction; but with southern pine this extraction may remove as high as two-thirds of the total extractable matter. With southern pine the extract so obtained is, or may be, a source of considerable profit since it contains turpentine, pine oil and a good grade of rosin. Stopping the extraction at this point gives much better rosin than if extraction be continued until all, or substantially all, of the resinous matter is removed.

While many other solvents may be employed in this partial extraction I find that described by Clope (Patent No. 1,144,171 June 22, 1915) on the whole is best adapted for my purposes. Clope uses a distillate from pine extracts distilling over between the turpentine fraction and the pine oil fraction. This solvent is a product of the process itself and its use imports nothing foreign into the material extracted thereby.

In the partial extraction of the chips a number of important advantages are secured. Firstly, of course, is the reduction of the resin content to a standard amount. Secondly, the chips are opened up to the penetration of the digestor liquors and made uniform in this way. In an unextracted chip of southern pine some cells are full of resinous matter and aqueous liquids penetrate only slowly while other cells are more pervious. In the partial extraction all the cells are made readily permeable; and the cells originally non-resinous now contain resin while those originally full of it, are

partially emptied; or, in other words, the resinous matter becomes equally distributed throughout the chip; and also from chip to chip of the charge. The whole charge in the extractor is made, more or less, uniform. With this equalizing of resin content comes an equalization of moisture. The chips are readily brought to a standard moisture content (usually about 20 per cent) by exposure to a damp atmosphere; or by a slight drying in the event that after extraction steam has been used to remove residual solvent, as is usually the case. The chips tend to retain this standard moisture content without much variance by exposure to the atmosphere. The extraction, further, leaves the chips somewhat porous and compressible, rendering it easy to bale them under pressure; and in bales the standard moisture content is of course still more easily preserved.

In standardizing the resin content, the acid content of the wood is also standardized; that is, the amount of soda which will be neutralized in the digestor is made standard.

With chips made as described, the paper maker is given a material containing a known and constant amount of moisture; a known amount of resins; and a known acid value. Within limits, the chip can be produced from almost any kind of pine or coniferous wood and be given the same standard composition.

In a specific embodiment of my invention, southern pine in any form (light wood, stumps, saw mill waste, etc.) is cut into pulp makers' chips and given a brief extraction in any suitable form of extractor. Clope's solvent may be used advantageously. With most of this material when about 70 per cent of the extractable matter is removed, there is a sudden increase in the difficulty of extraction; probably because of the low capillary powers of the residual more or less gummy and amorphous terpenes and resins. After the extraction, residual solvent is removed as by steaming in the usual way. Steaming at this stage probably contributes material to the described equalization of residual resinous matter. The steamed chips are then given a slight drying to bring the moisture to a standard amount, usually about 20 per cent, and are then baled.

The mill size long fibred partially extracted chips which form the subject of this invention may be and preferably are produced directly in the woods,—that is at the source and shipped from there to the pulp mill. This is of advantage both to the field operator and to the mill, in that it means that the wood can be inexpensively reduced to mill size and made ready for the pulp mill in the woods without requiring at this point either complicated expensive machin-

ery or much skilled labor for its operation. The pulp mill by this means receives long fibred mill size chips ready, without further treatment, to go directly to the digesters and forming a standard stock.

By means of my invention it will be seen that the pulp manufacturer is for the first time in the history of the art supplied with a standardized material suitable for the manufacture of high grade pulp and one which can be relied upon to produce uniform and satisfactory results.

By reason of the fact that the chips are free of the greater portion of turpentine and resinous constituents, the alkali necessary for the pulping treatment is less than has been usually required and with the moisture content known and running substantially uniform, as it does, the amount of alkali for given results can be readily predetermined. Because of the uniform distribution of the resin content in the chips, the chemicals used in cooking will act upon all of the chips to the same degree.

With such an extraction as is above described neither the extracts nor the chips are injured or stained materially by the metal of the apparatus, nor is either the wood or resinous material injured by long heating.

Such turpentine and other volatile terpenes as are not extracted by the solvent in the first operation, may, in a large measure, be recovered from the waste gases of the digester.

In an application, Serial No. 405,964 filed herewith, I have described and claimed a process similar to that disclosed herein for producing pulp mill chips from resinous woods, and in another application, Serial No. 405,963, also filed herewith, I am claiming the process of recovering the valuable products from resinous wood by first subjecting it to a volatile solvent to remove some of the extractives, pulping it with an alkaline solution and recovering the residual resinous matters from the spent alkaline solution.

What I claim is:—

1. As a new material, a pulp mill chip containing a substantial quantity of resinous matter, the amount however being substantially less than that normal to the wood and being distributed with greater uniformity,

said chip being open and porous in texture but not changing substantially in moisture content on exposure to the air.

2. As a new material, a pulp mill chip of resinous coniferous wood containing a substantial quantity of resinous matter, the amount however being substantially less than that normal to the wood and being distributed with greater uniformity; said chip being open and porous in texture but not changing substantially in moisture content on exposure to the air.

3. As a new material for pulp maker's purposes, a bale of pervious open textured coniferous wood chips, said chips containing a substantial amount of resinous material, but having sufficient of their normal resinous content removed to render them easily compressible, said bale being of standardized moisture content and said chips being assembled therein under pressure.

4. As a new material for pulp maker's purposes, a bale of pervious open textured southern pine wood chips, said chips containing a substantial amount of resinous material, but having sufficient of their normal resinous content removed to render them easily compressible, said bale being of standardized moisture content and said chips being assembled therein under pressure.

5. As a new material, pulp mill chips of coniferous wood having the resinous content thereof reduced but having a substantial residual resinous content distributed to render the texture of said chips substantially uniform.

6. As a new material, pulp mill chips of coniferous wood having the resinous content thereof reduced but having a substantial residual resinous content distributed to render the texture of said chips substantially uniform, and having a standardized moisture content.

7. As a new material, pulp mill chips of coniferous wood having the resinous content thereof reduced but having a substantial residual resinous content distributed to render the texture of said chips substantially uniform, having a standardized moisture content and baled to preserve the moisture content.

In witness whereof, I have hereunto set my hand this 23d day of August, 1920.

JOSEPH H. WALLACE.